

1

3,257,205

### METHOD FOR HEAT DEVELOPMENT

Paul Maria Cassiers, Mortsel-Antwerp, Louis Maria De Haes, Edegem-Antwerp, Gerard Laurens Vanreusel, Mortsel-Antwerp, and Josef Frans Willems, Wilrijk-Antwerp, Belgium, assignors to Gevaert Photo-Producenten N.V., Mortsel, Belgium, a Belgian company  
No Drawing. Filed Oct. 10, 1961, Ser. No. 147,388  
Claims priority, application Netherlands, Oct. 12, 1960,  
256,771

5 Claims. (Cl. 96—29)

This invention relates to an improved method for the manufacture of photographic images by a "dry" processing of photographic silver halide emulsions and to material for the application of this method.

It is known from the German patent specification 888,045 that photographic layers can be obtained which are developable by heat, by incorporating into silver halide emulsions substances which reduce silver halide salts, such as hydrazine, phenyl hydrazine, acid hydrazides, semicarbazides, methyl-p-aminophenol sulphate, hydroquinone and pyrocatechol.

Other suitable reducing compounds for heat development processes are aromatic amino-, hydroxy-, and amino-hydroxy-compounds and their derivatives, many examples of which are described in German patent specification 895,101 and Belgian patent specifications 544,850, 545,042 and 555,103.

The use of the developing substances, however, which are described in these patent specifications, involved various disadvantages. Especially the keeping quality of such emulsions before exposure leaves much to be desired.

Also the image obtained is of an inferior quality because of the too low density and the too soft gradation of the light-sensitive material.

According to the present invention a process has been found for the production of photographic images by heat-development, wherein a photographic material comprising a silver halide emulsion layer and incorporated in this silver halide emulsion layer and/or in a layer adjacent thereto, a 3-pyrazolidone compound of the formula



wherein:

$\text{R}_1$  represents a hydrogen atom, an aryl radical or a substituted aryl radical;

$\text{R}_2$  represents a hydrogen atom or an acyl radical;

each of  $\text{R}_3$ ,  $\text{R}_4$ ,  $\text{R}_5$  and  $\text{R}_6$  (equal or different) represents a hydrogen atom, an alkyl radical, a substituted alkyl radical, an aryl radical or a substituted aryl radical,

after or during exposure to an object to be reproduced, is subjected to a heat treatment, the pH of the silver halide emulsion during the heat-development being 7 or less.

Some compounds according to the present invention, which appeared from the experiments to give particularly

2

good results when used in this new method, are identified hereinafter:

- 1-phenyl-3-pyrazolidone
- 5 1-(m-tolyl)-3-pyrazolidone
- 1-phenyl-2-acetyl-3-pyrazolidone
- 1-phenyl-4-methyl-3-pyrazolidone
- 1-phenyl-5-methyl-3-pyrazolidone
- 1-phenyl-4,4-dimethyl-3-pyrazolidone
- 10 1-phenyl-5,5-dimethyl-3-pyrazolidone
- 1,5-diphenyl-3-pyrazolidone
- 1-(m-tolyl)-5-phenyl-3-pyrazolidone
- 1-(p-tolyl)-5-phenyl-3-pyrazolidone
- 5-phenyl-3-pyrazolidone

15 The developing substances according to this invention may be incorporated, either into the silver halide emulsion or into a separate adjacent layer.

The best known of these developing substances viz. 1-phenyl-3-pyrazolidone on itself possesses only poor developing properties as far as development in aqueous medium is concerned (J. D. Kendall, Brit. J. Phot. (1951) 539). It is really surprising that these substances, even when used in the absence of any other developing substance, possess a high developing power if used in a photographic material subjected to heat-development. Still more unexpected is the fact that this strong developing power even occurs not only in neutral and weak acid medium, but even in relatively strong acid medium, e.g., of pH 4.5.

20 30 The developability of the above described silver halide emulsions can still be improved by incorporating into these emulsions compounds which on heating liberate water.

35 The use of hydrophilic plasticizers, e.g., glycerol, caprolactam, polyethylene glycol and the like, also results into an improvement of the heat-developability. Also in this kind of emulsions the image quality can be improved by incorporating into the emulsions compounds which favorably influence the image tone, e.g., 1-phenyl-5-mercapto-tetrazole or similar products, which are described in British patent specification 561,875 and Belgian patent specification 502,525.

40 45 An advantage of the new process is the excellent quality of the produced images with regard to the density as well as in respect of the gradation. After rinsing and fixing, the obtained density is also much better kept than it is in the case with the most known developing substances.

A second advantage is the short developing time: in some cases the development has to last for only 1 to 10 50 sec. at a temperature between 100 and 200° C. Furthermore, the material according to the invention has very good keeping properties before its exposure, as derivatives of 1-phenyl-3-pyrazolidone in a non-alkaline medium and a normal temperature show but a poor reactivity.

55 60 A further advantage is the broad thermal margin of working up of the silver halide emulsions which are prepared with these new compounds. It has been experienced that the temperature fluctuations during the heat-development may amount to 30 to 40° C. without incurring the risk that less good images are obtained.

The amount of warmth which is necessary for the development may be applied onto the material in various

ways. So the silver halide emulsion can be developed by conduction, by contacting it with heated plates or rollers, by placing it between two capacitor plates which are subjected to a high frequency field, or by subjecting it to the Joule effect. The silver halide emulsion can also be developed by convection, e.g., by contacting it with directed warm gas stream. For this purpose, e.g., warm air or steam may be used. Finally the silver halide emulsion can also be developed by warmth radiation. The use of infrared radiation sources is especially suited therefore, not only because they have an intensive developing power, but also because they enable simultaneously to expose and to develop in a fraction of a second. By infrared radiation sources those radiation sources are understood of which the major part of the radiated energy waves possess a wave-length of  $10^{-4}$  to  $10^{-1}$  cm. In this way it is possible to contact a light-sensitive material, prepared according to this invention, with a film negative and to move it along a light-source which is rich in infrared radiations so as to obtain immediately a very strong positive image.

An especially interesting embodiment of this invention is the manufacture of prints of the heat-developed images according to the transfer process, which is described in the German patent specification 895,101. As is described in that German patent specification the silver halide layers which are developable by heat, contain a developing substance which, by reduction of the silver halide to silver on the exposed image areas, is used up and which on the unexposed image areas diffuses under the influence of the supplied warmth into an image-receiving layer brought into contact with the silver halide emulsion layer.

Analogously the process according to the present invention can be carried out by contacting the negative layer containing the developing substance, before the heat-development, with a positive layer containing a colorless triazolium compound of the general formula



wherein:

each of R<sub>7</sub> and R<sub>8</sub> (equal or different) represents an aliphatic group, a substituted aliphatic group, a homocyclic group, a substituted homocyclic group, a heterocyclic group, or a substituted heterocyclic group;

X represents an acid radical, and

Y represents the necessary atoms for closing an homocyclic group, substituted homocyclic group, a heterocyclic group, or a substituted heterocyclic group.

Such triazolium compounds are described, e.g., in French patent specification 998,055.

According to another embodiment of the present invention, the negative layer is contacted, before the heat-development, with a positive layer which contains a colorless tetrazolium compound of the formula:



wherein:

each of R<sub>9</sub>, R<sub>10</sub> and R<sub>11</sub> (equal or different) represents an aryl group or a substituted aryl group.

Such tetrazolium compounds can be prepared, e.g., according to the method described in British patent specification 670,883.

Some triazolium compounds according to the above Formula II which appeared from the experiments to give particularly good results are, e.g., 2,3-diphenyl-naphtho-

(1,2)triazolium chloride and 2-phenyl-3-(o-carboxyphenyl)-naphtho(1,2)triazolium chloride.

Some tetrazolium compounds according to the above Formula III which appeared from the experiments to give particularly good results are, e.g., 2,5-diphenyl-3-(o-carboxyphenyl)-2,1,3,4-tetrazolium chloride, 2,5-diphenyl-3-(o-methoxyphenyl)-2,1,3,4-tetrazolium chloride and 2,5-diphenyl-3-(p-methoxyphenyl)-2,1,3,4-tetrazolium chloride.

10 The development substances which remained unused during the heat-development, diffuse into the positive layer and there reduce the above mentioned colorless triazolium and tetrazolium compounds to dyes. The color tone, the fastness to light and the fastness to washing of these dyes can markedly be improved by the presence in the positive material of salts of multivalent metals, e.g., zinc, copper, iron, cadmium, cobalt, nickel, chromium, titanium, molybdenum, or tungsten, if tetrazolium compounds are used wherein R<sub>9</sub> is an aryl radical, which in its ortho position bears an electronegative group such as a carboxyl group.

15 Another interesting embodiment of this invention is based on the formation of a silver image in the positive material. For this purpose, the exposed negative is contacted during the heat-development with a positive material containing silver salts, e.g., silver nitrate. The developing substances which remain unused during the heat-development diffuse into the positive layer and there reduce the silver salts into metallic silver.

20 The following examples illustrate the invention without limiting, however, the scope thereof. The silver halide emulsion layers in the dried light-sensitive materials preferably contain per sq. m. 3 g. of gelatin and an amount of silver halide corresponding to 1 g. of silver.

#### Example 1

A photographic paper support of 90 g./sq. m. is coated with a layer from a suspension of the following composition:

|    |                                   |                  |      |
|----|-----------------------------------|------------------|------|
| 40 | Silver chloride emulsion          | g                | 1000 |
|    | Water                             | cm. <sup>3</sup> | 465  |
|    | Ethanol                           | cm. <sup>3</sup> | 400  |
|    | 1-phenyl-3-pyrazolidone           | g                | 25   |
|    | Glycerol                          | g                | 100  |
|    | Saponine                          | g                | 5    |
| 45 | 40% aqueous formaldehyde solution | cm. <sup>3</sup> | 5    |

50 This paper is then dried, exposed through an original and heat-developed either by contacting this paper with a plate heated at 80-200° C. or by treating it with a steam jet of 100° C. A sharp print of the original is obtained. This print may be fixed and stabilized according to known processes.

#### Example 2

A photographic paper support of 90 g./sq. m. is coated with a layer from a suspension of the following composition:

|    |                                   |                  |      |
|----|-----------------------------------|------------------|------|
| 60 | Silver bromide emulsion           | g                | 1000 |
|    | Water                             | cm. <sup>3</sup> | 465  |
|    | Ethanol                           | cm. <sup>3</sup> | 400  |
|    | 1-phenyl-3-pyrazolidone           | g                | 25   |
|    | Caprolactam                       | g                | 100  |
|    | Saponine                          | g                | 5    |
| 65 | 40% aqueous formaldehyde solution | cm. <sup>3</sup> | 5    |

65 After further treatment, exposure and heat-development as in Example 1, a sharp print of the original is obtained.

#### Example 3

A photographic paper support of 90 g./sq. m. is coated with a layer from a suspension of the following composition:

|    |                                  |                  |      |
|----|----------------------------------|------------------|------|
| 70 | Silver chloride emulsion         | g                | 1000 |
|    | Water                            | cm. <sup>3</sup> | 465  |
|    | Ethanol                          | cm. <sup>3</sup> | 400  |
| 75 | 1-phenyl-4-methyl-3-pyrazolidone | g                | 25   |

## 5

|                                                                                                                                        |                  |     |
|----------------------------------------------------------------------------------------------------------------------------------------|------------------|-----|
| Carbowax 200 (trade name of Union Carbide and Carbon, New York, N.Y., for a polyethylene glycol of an average molecular weight of 200) | g.               | 100 |
| Saponine                                                                                                                               | g.               | 5   |
| 40% aqueous formaldehyde solution                                                                                                      | cm. <sup>3</sup> | 5   |
| 1% solution of 1-phenyl-5-mercapto-1,2,3,4-tetrazole in ethanol                                                                        | cm. <sup>3</sup> | 100 |

After further treatment, exposure and heat-development as in Example 1, a sharp print of the original is obtained.

## Example 4

A negative material is prepared by coating a paper support of 90 g./sq. m. with a layer from a suspension of the following composition:

|                                   |                  |      |
|-----------------------------------|------------------|------|
| Silver chloride emulsion          | g.               | 1000 |
| Water                             | cm. <sup>3</sup> | 1000 |
| Glycerol                          | cm. <sup>3</sup> | 100  |
| Saponine                          | g.               | 5    |
| 40% aqueous formaldehyde solution | cm. <sup>3</sup> | 2    |

This layer is applied in such a way that 1 l. of this suspension covers 10 sq. m. of paper. Upon this layer is then applied a layer from the following solution:

|                         |                  |      |
|-------------------------|------------------|------|
| Ethanol                 | cm. <sup>3</sup> | 1000 |
| 1-phenyl-3-pyrazolidone | g.               | 50   |

This layer is applied in such a manner that 1 l. of this solution covers 20 sq. m. of paper.

A positive material is prepared by dip-coating a paper support of 90 g./sq. m. with a 0.1% aqueous silver nitrate solution and drying it.

The silver halide emulsion side of the negative material, in contact with the original, is reflectographically exposed. The negative material is pressed for about 5 sec. with its emulsion side against the prepared positive material by means of a flat-iron at about 150° C.

The part of developing substance which during the heat-development did not serve to reduce the silver halide into silver, diffuses onto the positive layer and reduces the silver nitrate into silver. A clear print of the original is obtained.

## Example 5

A photographic paper support of 90 g./sq. m. is coated with a layer from a suspension of the following composition:

|                                                                 |                  |     |
|-----------------------------------------------------------------|------------------|-----|
| Silver chloride emulsion                                        | cm. <sup>3</sup> | 100 |
| Water                                                           | cm. <sup>3</sup> | 10  |
| Ethanol                                                         | cm. <sup>3</sup> | 5   |
| 1-phenyl-3-pyrazolidone                                         | g.               | 1   |
| Potassium metabisulfite                                         | g.               | 1   |
| Sodium acetate                                                  | g.               | 20  |
| 99% acetic acid                                                 | cm. <sup>3</sup> | 3   |
| Saponine                                                        | cm. <sup>3</sup> | 0.5 |
| 40% aqueous formaldehyde solution                               | cm. <sup>3</sup> | 0.5 |
| 1% solution of 1-phenyl-5-mercapto-1,2,3,4-tetrazole in ethanol | cm. <sup>3</sup> | 2.5 |
| Titanium dioxide                                                | g.               | 6   |

This layer is applied in such a way, that 1 l. of this suspension covers 10 sq. m. of paper.

A positive material is prepared by coating a paper support of 90 g./sq. m. with a layer from a solution of the following composition:

|                                                                                        |                  |     |
|----------------------------------------------------------------------------------------|------------------|-----|
| 5% aqueous solution of gelatin                                                         | cm. <sup>3</sup> | 50  |
| 15% aqueous solution of 2,5-diphenyl-3-(p-methoxy-phenyl)-2,1,3,4-tetrazolium chloride | cm. <sup>3</sup> | 20  |
| 10% aqueous solution of cupric sulfate                                                 | cm. <sup>3</sup> | 5   |
| 20 g. of anhydrous sodium acetate dissolved in water to                                | cm. <sup>3</sup> | 24  |
| 10% aqueous formaldehyde solution                                                      | cm. <sup>3</sup> | 0.5 |

The negative material is reflectographically exposed to a printed original and developed by pressing it for 10 sec. against a heated plate at 110° C. Then the developed

75

## 6

negative material is contacted with the positive material for 20 sec. at 110° C. After separation of the materials, a strong red print of the original is obtained onto the positive material.

## Examples 6-7

Similar results are obtained by replacing in the above solution the 2,5-diphenyl-3-(p-methoxyphenyl)-2,1,3,4-tetrazolium chloride by a same amount of 2,5-diphenyl-3-(o-methoxyphenyl)-2,1,3,4-tetrazolium chloride or 2,3-diphenylnaphtho (1,2)triazolium chloride.

We claim:

1. A process for the production of photographic copies by heat development which comprises the steps of:

(1) Exposing to the object to be copied a photographic material comprising a silver halide emulsion layer and containing a compound liberating moisture on heating and a 3-pyrazolidone developing compound of the general formula:



wherein:

$R_1$  is a member of the group consisting of hydrogen and an aryl radical,

$R_2$  is a member of the group consisting of hydrogen and an acyl radical, and

$R_3$ ,  $R_4$ ,  $R_5$  and  $R_6$  are each a member of the group consisting of hydrogen, an alkyl radical and an aryl radical;

(2) Developing said exposed emulsion layer by subjecting said layer to a heat treatment at a pH of not more than 7 while said material is maintained in effective separable contact with an image-receiving layer containing an initially colorless image-forming compound selected from the group consisting of (1) silver nitrate, (2) a triazolium compound having the general formula:



wherein:

$R_7$  and  $R_8$  are each a member of the group consisting of an aliphatic group, a homocyclic group, and a heterocyclic group,

$X$  is an acid radical, and

$Y$  represents the atoms necessary for closing a ring of the group consisting of a homocyclic ring and a heterocyclic ring;

and (3) a tetrazolium compound having the general formula:



wherein:

$R_9$ ,  $R_{10}$  and  $R_{11}$  are each an aryl group.

2. The process of claim 1 wherein said developing compound is incorporated in said emulsion layer.

3. The process of claim 1 wherein said moisture-liberating compound is incorporated in said emulsion layer.

4. The process of claim 1 wherein said exposure and development steps are carried out concurrently.

5. The process of claim 1 wherein said emulsion layer is exposed to a radiation source rich in infrared rays while in contact with the object to be copied.

(References on following page)

## References Cited by the Examiner

## UNITED STATES PATENTS

|           |         |                |        |
|-----------|---------|----------------|--------|
| 2,751,297 | 6/1956  | Hood et al.    | 96—109 |
| 2,751,300 | 6/1956  | James et al.   | 96—29  |
| 2,891,862 | 6/1959  | Allan          | 96—109 |
| 2,971,840 | 2/1961  | Hydn et al.    | 96—29  |
| 3,007,795 | 11/1961 | Hydn et al.    |        |
| 3,015,562 | 1/1962  | Herrick et al. | 96—29  |
| 3,041,170 | 6/1962  | Haist et al.   | 96—95  |
| 3,042,514 | 7/1962  | Roth           | 96—29  |

## FOREIGN PATENTS

|           |        |                |
|-----------|--------|----------------|
| 530,883   | 8/1954 | Belgium.       |
| 554,934   | 8/1957 | Belgium.       |
| 998,055   | 1/1952 | France.        |
| 1,003,578 | 9/1952 | Germany.       |
| 670,883   | 4/1952 | Great Britain. |
| 845,928   | 8/1960 | Great Britain. |

NORMAN G. TORCHIN, Primary Examiner.  
 LOUISE P. QUAST, Examiner.  
 J. T. BROWN, Assistant Examiner.